

C. A. WEEKS,  
ELECTRIC FURNACE,  
APPLICATION FILED OCT. 23, 1909.

1,034,747.

Patented Aug. 6, 1912.

3 SHEETS—SHEET 1.



FIG. 2



FIG. 1

1,034,747.

C. A. WEEKS.  
ELECTRIC FURNACE.  
APPLICATION FILED OCT. 23, 1909.

Patented Aug. 6, 1912.

3 SHEETS--SHEET 2.



1,034,747.

C. A. WEEKS.

ELECTRIC FURNACE.

APPLICATION FILED OCT. 23, 1909.

Patented Aug. 6, 1912.

3 SHEETS-SHEET 3.



FIG. 4

WITNESSES

E. J. Farley  
J. M. Cunningham

INVENTOR  
Charles A. Weeks  
BY  
*Charles A. Weeks*  
ATTORNEY

# UNITED STATES PATENT OFFICE.

CHARLES A. WEEKS, OF PHILADELPHIA, PENNSYLVANIA.

## ELECTRIC FURNACE.

1,034,747.

Specification of Letters Patent.

Patented Aug. 6, 1912.

Application filed October 23, 1909. Serial No. 524,240.

To all whom it may concern:

Be it known that I, CHARLES A. WEEKS, a citizen of the United States, and a resident of the city and county of Philadelphia, 5 State of Pennsylvania, have invented an Improvement in Electric Furnaces, of which the following is a specification.

My invention has reference to electric furnaces and consists of certain improvements 10 which are fully set forth in the following specification and shown in the accompanying drawings which form a part thereof.

The object of my invention is to provide a suitable construction of furnace adapted 15 to the employment of the high temperature of an electric arc for the smelting of copper, iron and other ores both for the purpose of reducing and refining.

More particularly the object of my invention is to provide a furnace in which the reducing and refining operations may be carried on in a continuous manner and at a 20 minimum expense, and, moreover, under absolute control as to temperature and character of reducing gases.

My object is also to reduce the time necessary in which the reduction of the ores and refining of the metal may take place, thereby cheapening the cost; and also to enable 30 the refinement to be done under a high temperature which is capable of satisfactorily treating the most refractory materials.

The general character of my improved furnace comprehends the employment of a 35 long, slightly inclined tubular rotary reducing flue, terminating at its highest end in the chimney and ore feeding device, and communicating at its lower end with an electric furnace so constructed as to have 40 provisions for rocking or otherwise moving its hearth while maintaining communication with the tubular flue, and combining with such structure means for providing a reducing or other flame in that portion of the 45 tubular flue adjacent to its lower end for completing the reduction of the ores before the metal is delivered to the hearth of the electric furnace in which the refining is performed.

50 In the preferred construction of my improved furnace I support the electric furnace proper by means of curved rockers guided upon suitable supporting rollers and rocked by means of mechanical power and 55 in which the axis about which the furnace rocks is concentric or substantially concen-

tric with the lower end of the rotating tubular flue and with which communication is made by means of a connecting flue or neck secured and moving with the said electric 60 furnace proper.

My invention more fully consists of constructions which are described in the following specification and more particularly defined in the claims; and these improvements 65 will be better understood by reference to the drawings, in which:

Figure 1 is a side elevation of my improved furnace, complete; Fig. 2 is a plan view of the same on a larger scale, with a 70 large portion of the rotary flue broken away; Fig. 3 is a sectional elevation of the same; and Fig. 4 is a cross section through the electric furnace.

2 is a long sheet metal flue built of sections and lined with fire brick or suitable refractory material; and at intervals in its length it is provided with circular bearings 3 which run upon supporting rollers 4, whereby the flue, as a whole, may be freely 80 rotated. The bearings are supported upon pedestals 5 and these are gradually reduced in height so that one end of the tubular flue 2 is supported at a higher elevation than the other or lower end, said inclination 85 being adapted to cause the ore and fluxes to gradually work downwardly through the flue during its rotation, and to cause the gas to pass upward through the same or in a reverse direction. This rotary flue 2 may 90 be rotated by means of an electric motor 8, a variable speed gear 7 and an annular gear 6 surrounding the cylinder of the tubular flue 2. By means of the variable gearing 7, the speed of rotation of the flue may be 95 made commensurate with the requirements, but I do not limit myself to any particular speed. The flue may be rotated in any suitable manner desired.

9 is the receiving chamber for the gases 100 passing from the flue 2 and is provided with a tubular opening 16 into which the end of the flue extends, as clearly shown in Fig. 3. Opening from this chamber 9 is the chimney 10 which may be provided with a suitable 105 damper 11 which controls the amount of draft. At the bottom of the chamber 9 is a cleanout door 12 through which the heavy deposit collected in the chamber may be removed. A flue 40 may open from the chamber 110 9 for conveying the gas to the gas engine or the furnace for heating the boilers

when the waste gases are free from substances which it is desirable to collect; but in the case where the gases are sulfurous, the said flue 40 may be connected with textile bags 41 in which the sulfur is collected. 5 Any other desirable use of the escaping gas from the flue 40 may be employed, if so desired.

17 is the electric furnace and consists of a 10 large body part having an obliquely extending neck 21 terminating in a head 22 provided with plates 23 having a tubular opening into which the lower end of the tubular flue 2 extends, as shown in Fig. 3. 15 This head 22 opposite to the end of the flue 2 is provided with a door 24 through which a nozzle 25 extends for providing a blast of air, gas or fuel in subdivided form, the gas or fuel required being varied to suit 20 the particular character of the ores to be reduced in their passage through the rotary flue 2. The electric furnace is supported upon curved rockers 18, the curvature of which is struck from the axis corresponding 25 to the center of the opening in the plates 23 of the head of the furnace and therefore concentric with the center of the lower end of the flue 2 adjacent to this point. These rockers 18 rest upon supporting rollers 19 30 carried upon the bed plate and foundations. The furnace may be rocked in any suitable manner, but in the particular structure shown, this is accomplished by cylinders and pistons 20 of any ordinary construction and 35 which may be operated by steam, air or otherwise and under any suitable controlling means. The furnace may be rocked by any other mechanism, if so desired.

More particularly, the furnace is 40 constructed of a sheet iron shell supported on the bottom on a series of longitudinal I beams 35 which rests upon the rockers 18 and the shell is reinforced over its upper part by a series of curved beams 36. The 45 sheet iron shell is lined with suitable refractory material 28 and preferably provided with a magnesite hearth 27. The interior part of the roof over the hearth is curved in transverse sections, as indicated 50 in Fig. 4 and substantially straight in longitudinal section, as indicated in Fig. 3. The hearth 27 is preferably curved downward at the middle approximately parallel with the curvature of the rockers 18 and has the 55 ends curved upward so that the general cross section of the interior of the furnace is elliptical. Each side of the furnace is provided with one or more, electrodes 29, which are carried by water cooled bushings 60 and through which these electrodes are fed to compensate for their consumption. The water may be supplied to the bushing in any suitable manner. These electrodes on opposite sides are arranged at an angle to each other, as indicated in Fig. 4, so as to

cause the arc between them to be presented close to the surface of the metal upon the hearth. The electrodes may be fed through cooled jackets 30 in any suitable manner, but as indicated, are adjustable by gearing 70 31 for each electrode and connected by a transverse power shaft 32 which is rotated by worm and worm-wheel gearing 33 operated by a suitable electric or other motor 34. By rotating the shaft 32 in one direction or the other, the electrodes 29 may be advanced or retracted and in this manner the length of the arc between the opposite electrode maintained, as may be required. The electrode feeding mechanism is carried with the electric furnace 17 and these are rocked together, as a unit. The neck 21 as well as the hearth 27 may be lined with magnesite and especially, that portion of the neck over which the metal flows in passing from the flue 2 to the hearth 27. The refined metal may be drawn off through a tapping hole 37 and the slag may be run off through the tapping hole 38 also in front of the furnace, but at a higher elevation. 80

It will be understood that the electric furnace used in refining, may be of any length desired and provided with one, two or more pairs of electrodes, dependent upon the capacity of the furnace, and I therefore 95 do not limit myself to the use of a plurality of pairs of electrodes.

The ores to be treated in my improved furnace are first pulverized and fed into a hopper 13 and from this hopper the pulverized ore passes into an oblique chute 14 and, by means of a feeding screw 15, is delivered into the upper end of the tubular rotary flue 2, as shown in Fig. 3. If desired, the extreme upper end of the lining of the 100 flue 2 may be thickened, so as to reduce the tubular outlet to a diameter considerably less than the diameter at the remaining portion of the flue, as clearly indicated. The means for supplying fuel, either in gas or 105 pulverized form to the lower end of the flue 2, may be of any character desired and that shown at 25 is only given by way of illustration. The particular character of burners for this purpose would be especially designed for the character of work to be done in the furnace and may vary in the same furnace when applied to the smelting of 110 different ores. 115

26 is a valve to control the fuel supplied by the burner 25. The fuel supplied by the nozzle or burner 25 is usually of a reducing character, so that in passing through the flue 2, in the reverse direction to the travel of the crushed ores, the latter will be reduced gradually from the time of its entrance into the rotary flue and throughout its travel toward the lower end thereof or into zone of dissociation and preliminary to the flow of the metal formed down the neck 120 125 130

21 into the electric furnace. On the other hand, the electric furnace is adapted to treat the crude metal that is produced in the rotary flue to the intense heat of the electric 5 arc and reverberatory action of the heat energy, without special requirements either as to reducing or oxidation. In this furnace 17, the metal is refined by a high temperature and the lighter slags are caused to 10 separate and rise to the surface of the molten metal. The refining action in the electric furnace is facilitated by the oscillation thereof, which causes the molten metal to be constantly disturbed and thereby enabled 15 to free itself of objectionable slags and unreduced elements which may be contained therein when delivered to the hearth. In the oscillation of the electric furnace 17, the head 22 thereof at all times maintains its 20 connection with the lower end of the rotary flue 2, because of the fact that the curvature of the rockers 18 are struck from a center in axial alinement through the axis of the rotary flue where it enters the head 22 of the 25 neck of the electric furnace.

In using my improved furnace in the smelting of iron ores for the manufacture of iron and steel, substantially the same reactions take place in the apparatus as take 30 place in a blast furnace but with more satisfactory results and with more positive action as to final outcome and product. Assuming that proper pulverized mixture of sesquioxid of iron and lime stone were fed 35 into the upper end of the flue 2 from the hopper 13, we would have essentially the following reactions if it be understood that the gases which are fed in from the nozzle 25 were produced from carbon. If we assumed that pulverized carbon be injected 40 with the proper air and supplemented by the high temperature rising from the electric furnace through the neck 21 thereof, we will have a very high temperature in the 45 lower part of the flue 2 and a gradually lessening temperature as we approach the stack end. The ores, mixed with carbon and limestone, delivered in the upper end of the rotary flue, are reduced at a dull red heat 50 by the carbon-monoxid gases and as the materials pass therefrom down the flue the lime-stone is decomposed, giving off carbonic acid, which, by combination with carbon, forms carbon-monoxid and assists in 55 the reduction of the iron oxid. At a full red heat, farther down the furnace, the carbon-monoxid is decomposed, producing carbon deposit which is absorbed by the iron at about a temperature equal to bright red. 60 After the carbon deposition and absorption by the iron we have cast iron or steel according to the amount of carbon absorbed and this may be regulated by the control of the relative amount of carbon present in the 65 gas or mixture. The crude metal which is

thus produced is then subjected to a higher temperature equivalent to a very bright red heat and at this fusion takes place with gradual separation of slag. The mixture of metal and slag are then subjected to an increased temperature, equivalent to white heat and approximately from 2700 to 3000° Fh., where they enter the furnace 17 by the neck 21. Within this electric furnace the temperature may be raised to considerably over 3000° Fh. and thereby produce a clear separation of the slag and other impurities from the steel and which is treated to agitation when being subjected to higher temperature as an open hearth proposition. The slag may then be run off and finally the refined steel tapped from the hearth. 70 75 80

In practice, the fluxing and the proportion of carbon supplied, either from the nozzle 25 alone or by mixtures with the crushed ore, may be varied to suit the character of the iron to be treated, as these conditions would vary according as to whether the iron was red-hematite above mentioned as sesquioxid of iron, or iron ores such as brown-hematite and spathic iron ores. When the percentage of carbon reaches 1.4, the metal begins to assume the characteristics of cast iron and approximately from .5 to 1.5 may be taken as steel, as ordinary form of steel 90 approximately contains about 1.2 of carbon. It is further seen that some care in the action of the furnace will be necessary to cause proper carbon absorption to insure the desired grade of the refined steel. In a 95 furnace of this character, it is also possible to conveniently free the iron from sulfur and phosphorus whereby the finished steel will be free from these detrimental elements. 100 105

In using the furnace for smelting of copper ores, the reduction of the copper ore will be performed in the rotary flue 2 and the refining completed in the electric furnace, the operation of the apparatus being 110 varied somewhat according to the character of the ore, that is to say, whether it is of malachite, consisting of a composition of carbon and hydrated oxid of copper, a sulfuret of copper, or a red oxid of copper, for 115 example. The ores would be pulverized and fed into the rotary flue 2 from the hopper 13 and in the upper portion of the flue 2 they would be subjected to a reducing action. The sulfur, when present, passes off through the 120 chamber 9 and by flue 40 and collects in the textile bags 41. The metal regulus formed by the action of the gas in the rotary flue 2 during the passage of the copper ores through the same, will be essentially a mixture of copper, sulfuret of copper, and iron or other metals and is treated in the higher temperature zone to fusion and by the rotary action of the flue 2, is fed down into the electric furnace 17. During the reduc- 125 130

ing operation of the smelting within the flue 2 the sulfur is substantially eliminated and during this action the reduction may be performed largely by oxidation, according to 5 the requirements. If proper fluxing of the ores is done when supplied to the rotary flue, the copper may be separated freely from the slag so that the ore may be properly smelted by the time it passes through 10 the rotary flue and the metal separated freely from the slag by the time they reach the electric furnace, and in which the separation of the slag and copper is completed, 15 the refining of the copper taking place in the electric furnace because of its high temperature and capacity for agitation. During the reducing operation, which is essentially an oxidizing one, the regulus becomes black due to the oxidizing of iron and oxid 20 present, whereas the gas with other substances are conveyed off and the sulfur collected, as hereinbefore stated. The reduction of the ores is practically completed before the copper and slag enter the electric 25 furnace, so that nothing is required in such part, excepting high temperature with or without agitation as desired. When the operation is completed the slag is run off and then the refined copper thereof discharged 30 in the molten form.

The foregoing explanation as to the operation of my improved furnace is given by way of illustration only, to indicate its applicability to smelting action generally and 35 not by way of limitation with respect to its use. It will also be understood that the general details of construction may be generally varied without departing from the spirit of the invention, and I therefore do 40 not restrict myself to the details shown, although I prefer them in the actual construction and use of my invention.

Having now described my invention, what I claim as new and desire to secure by Letters Patent, is:

1. The combination of a cylindrical flue smelting furnace of great length arranged on an incline and having distinct zones of temperature for roasting and reducing the ores 50 and for melting the metals thereof, means to rotate the said smelting furnace, means for supplying ores to the upper end of the said furnace, and an electric refining furnace having a hearth of refractory material adjacent to and opening into the lower end of 55 the flue of the smelting furnace by a passage for guiding the molten metal into the hearth and also having electrodes of opposite polarity arranged above the hearth.

2. The combination of a cylindrical flue smelting furnace of great length arranged on an incline and having distinct zones of temperature for roasting and reducing the ores and for melting the metals thereof, 60 means to rotate the said smelting furnace, 65

means for supplying ores to the upper end of the said furnace, an electric refining furnace having a hearth of refractory material adjacent to and opening into the lower end of the flue of the smelting furnace by a passage for guiding the molten metal into the hearth and also having electrodes of opposite polarity arranged above the hearth, and blast means for supplying fuel in finely subdivided state into the lower end of the flue of the smelting furnace wholly in addition to the hot gases coming from the electric furnace. 70 75

3. In an electric furnace, the combination of a long inclined rotary flue in which ores are smelted having distinct zones of temperature for roasting and reducing the ores, and then melting the metals thereof, combined with a chimney at the upper end of the flue, means to positively feed the ores and fluxes into the upper end of the rotary flue and directly across the chimney passage, an electric furnace arranged at a lower level than the lower end of the rotary flue and having a hearth of refractory material, an inclined connecting flue for connecting the hearth of the electric furnace with the lower end of the rotary flue for guiding the fluid metal as smelted in the rotary flue into the hearth of the electric furnace without permitting it to drop unsupported, and means independent of the electric furnace for supplying a fuel into the lower end of the rotary flue for producing a smelting temperature therein. 80 85 90 95

4. In a furnace, the combination of a long inclined rotary flue, means to supply ores to the upper end of the rotary flue, means to rotate the flue, an electric furnace having a hearth at a lower level than the end of the rotary flue and connected with it, means to support and rock the electric furnace while maintaining connection with the rotary flue, and means to supply fuel into the lower end of the rotary flue. 100 105

5. In a furnace, the combination of a long inclined rotary flue, means to supply ores to the upper end of the rotary flue, means to rotate the flue, an electric furnace at a lower level than the end of the rotary flue and having a neck portion extending 110 upward to and forming an adjustable connection with the flue, and means for giving to the electric furnace a reciprocating motion while maintaining its connection with the flue. 115 120

6. In a furnace, the combination of a rotary flue arranged on an incline, a chimney in connection with the upper end of the rotary flue and provided with a damper, means to feed ores into the end of the rotary flue adjacent to the chimney, means to rotate the rotary flue, an electric furnace having its hearth in communication with the lower end of the rotary flue, and means for 125 130

supporting and rocking the electric furnace about the end of the rotary flue.

7. In a furnace, the combination of a rotary flue arranged on an incline, a chimney in connection with the upper end of the rotary flue and provided with a damper, means to feed ores into the end of the rotary flue adjacent to the chimney, means to rotate the rotary flue, an electric furnace having its hearth in communication with the lower end of the rotary flue, and a tubular neck connecting the hearth of the electric furnace with the lower end of the rotary flue, and means for supporting and rocking the electric furnace about the end of the rotary flue consisting of rockers under the electric furnace and rocking upon supporting rollers.

8. In a furnace, the combination of a rotary flue arranged on an incline, a chimney in connection with the upper end of the rotary flue and provided with a damper, means to feed ores into the end of the rotary flue adjacent to the chimney, means to rotate the rotary flue, an electric furnace having its hearth in communication with the lower end of the rotary flue and a tubular neck connecting the hearth of the electric furnace with the lower end of the rotary flue, means for supporting and rocking the electric furnace about the end of the rotary flue consisting of rockers under the electric furnace and rocking upon supporting rollers, and means for delivering a fuel into the lower end of the rotary flue.

35 9. The combination of an inclined rotary tubular smelting furnace of great length in which the ores are smelted to provide fluid metal, a chimney in communication with the higher end of the tubular smelting furnace, power devices for rotating the said smelting furnace, an electric refining furnace adjacent to and in direct communication with the lower end of the rotary tubular smelting furnace and having a hearth adapted 40 to receive the molten metal from the smelting furnace, and means independent of the electric furnace or products for delivering fuel from an outside source into the lower end of the rotary tubular smelting furnace 45 in addition to the heat directly delivered thereto from the electric furnace.

50 10. In a furnace, the combination of a rotary flue of great length in which the ores are smelted, a chimney in communication with one end of the flue, power devices for rotating the flue, an electric furnace in communication with the end of the rotary flue most distant from the chimney and constructed and supported to have a movement 55 of the hearth thereof independent of the movement of the rotary flue, and means separate from the furnace for delivering fuel from an outside source to the rotary flue in addition to the heat directly delivered 60 thereto from the electric furnace and said

65 delivery of heat and fuel being at a point adjacent to the connection of the electric furnace with the rotary flue.

7. In an electric furnace, the combination of an inclosed hearth having an upwardly extending tubular neck opening from one end and provided with rockers, a flue independent from the hearth and having adjustable communication with the neck thereof supports for the rockers of the inclosed hearth, means for rocking the inclosed hearth on the supports while maintaining communication with the flue, and electrodes extending into the hearth for maintaining one or more electric arcs 80 therein.

11. In an electric furnace, the combination of an inclosed hearth having an upwardly extending tubular neck opening from one end and provided with rockers, 85 a flue independent from the hearth and having adjustable communication with the neck thereof, supports for the rockers of the inclosed hearth, means for rocking the inclosed hearth on the supports while maintaining communication with the flue, electrodes extending into the hearth for maintaining one or more electric arcs 90 therein, and means carried with the rocking inclosed hearth for adjusting the electrodes.

12. In an electric furnace comprising an inclosed hearth having an upwardly extending tubular neck at one end having a lateral outlet at the upper end for escape of gases, and rockers under the hearth having 100 their curvature struck from an axial line through the lateral outlet from the neck, supports for the rockers, means for rocking the hearth and rockers upon the supports and electrodes extending through the 105 inclosed hearth for providing one or more electric arcs in the hearth.

13. An electric furnace comprising an inclosed hearth having an upwardly extending tubular neck at one end and having a 110 lateral outlet at the upper end for the escape of gases, and rockers under the hearth having their curvature struck from an axial line through the lateral outlet from the neck, supports for the rockers, means for 115 rocking the hearth and rockers upon the supports, electrodes extending through the inclosed hearth for providing one or more electric arcs in the hearth, and means for feeding the electrodes rocking with the inclosed hearth and electrodes.

14. An electric furnace comprising an inclosed hearth having an upwardly extending tubular neck at one end and having a 120 lateral outlet at the upper end for the escape of gases, and rockers under the hearth having their curvature struck from an axial line through the lateral outlet from the neck, supports for the rockers, means for 125 rocking the hearth and rockers upon the supports, electrodes extending through the inclosed hearth for providing one or more electric arcs in the hearth, and means for feeding the electrodes rocking with the inclosed hearth and electrodes.

15. In a furnace, the combination of a reducing smelting furnace through which the ores and fluxes are fed and smelted to

125 fluid metal, means for supplying carbonaceous fuel in subdivided condition from an outside source to the lower end of said smelting furnace, an electric refining furnace having a hearth of refractory material arranged at a lower level than the compart-

ment and also communicating directly with the smelting furnace whereby the molten metal may flow into the hearth of the electric refining furnace, and means for producing and maintaining one or more electric arcs in the electric furnace above the hearth thereof.

16. In a furnace, the combination of a reducing compartment through which the 10 ores and fluxes are fed, means for supplying carbonaceous fuel to the lower end of said compartment an electric furnace arranged at a lower level than the compartment and having a tubular neck communicating with the compartment through which the molten metal may flow into the hearth of the electric furnace, means for producing and maintaining one or more electric arcs in the electric furnace, means for rocking the 15 electric furnace relatively to the reducing compartment.

17. The herein described method of smelting ores which consist in subjecting the ores to be treated associated with the fluxes to 20 the simultaneous action of hot reducing gases of gradually increasing temperature while the said ores and fluxes are kept in a state of agitation by being continually rolled over and over upon themselves while 25 being fed in contact with the smelting gases and while traveling in contact with said gases from their coolest condition toward 30 their hottest condition and thereby separating the metal from the gangue and fluxes 35 by causing it to melt, transferring the molten metal under action of gravity to a

hearth of refractory material, subjecting the molten metal to the high temperature of an electric arc and at the same time keeping it in a state of agitation, and finally separating the refined metal from the slag. 40

18. The method of smelting and refining ores, which consists in first subjecting the ores and fluxes to agitation and a gradually increasing temperature to positively smelt 45 the ores and free the metal thereof in a fluid state, then causing said fluid metal thus formed to at once flow into an inclosed chamber, subjecting the metal agitation within the inclosed chamber, and while so 50 agitated subjecting it to the refining action of an electric arc.

19. A combined smelting and refining apparatus which consists of a rotating smelting furnace of great length and having a 55 greatly varying temperature therein for gradually reducing the ores and then changing the metal thereof to a fluid condition, combined with a refining electric furnace immediately adjacent to the discharge end 60 of the smelting furnace, and a flue through which the fluid metal may flow from the smelting furnace into the electric refining furnace and the gases from the electric refining furnace pass in a reverse direction 65 into the smelting furnace.

In testimony of which invention, I hereunto set my hand.

CHARLES A. WEEKS.

Witnesses:

E. G. FARLEY,  
R. M. KELLY.